

**1**

3,477,566

**PROCESS FOR THE ELECTROSTATIC SEPARATION OF THE SYLVITE (KCl) COMPONENT OF A MINERAL**

Hans Autenrieth, Hannover-Kirchrode, and Heinrich Wirries, Hannover, Germany, assignors to Kali Forschungs Anstalt GmbH, Hannover, Germany  
No Drawing. Filed Dec. 12, 1966, Ser. No. 600,711  
Claims priority, application Germany, Mar. 11, 1966,

K 58,696

Int. Cl. B03b 1/04

U.S. Cl. 209—9

5 Claims

**ABSTRACT OF THE DISCLOSURE**

A process for the electrostatic separation of mineral mixtures, and particularly to conditioned particulate crude potassium salts and the electrostatic separation thereof.

In particular embodiments of the present invention crude particulate potassium salt mixtures are treated with inorganic mineral acids or inorganic alkaline reacting substances before, during or after the particulate material is treated with organic conditioning agents, comprising anionic compounds which form negatively charged radicals that split off positive ions and thereby control the electrostatic charging of the particulate material.

**CROSS-REFERENCES TO RELATED APPLICATIONS**

Applicants claim priority under 35 U.S.C. 119 for application Ser. No. K 58,696 filed Mar. 1, 1966, in the Federal Republic of Germany.

**BACKGROUND OF THE INVENTION**

It is known that minerals containing crude potassium salts and many other mineral mixtures can be separated into their components electrostatically after being preconditioned, especially by organic compounds which by forming negatively charged radicals split off one or more protons or metal ions. By a suitable choice of conditioning agent, or by a combination of different conditioning agents, the electrostatic charging of the different mineral components can be controlled so that multiple-component systems are separated completely with high yield into individual mineral components of greater purity.

These prior art methods, conditioning agents and starting materials are fully set forth in German Patents 1,056,551, 1,061,713, 1,076,593, and 1,102,663, and the corresponding U.S. Patent 3,217,876, the disclosures of which are incorporated herein.

Autenrieth discloses in U.S. Patent 3,217,876 conditioning agents and the recycling and reconditioning of a portion of the particulate salt mixture.

The conditioning agents disclosed in the prior art patents are suitable for use in the present invention.

It is postulated that the conditioning does not depend, like a flotation process, on a selective application of the conditioning agent to the mineral components. On the contrary, the conditioning for electrostatic separation is made without selectivity. The selective distribution of electric charges to the individual minerals is decisively favored according to the specificity of the particular mineral by the application of the conditioning agent to the surface of the powdered mineral mixture.

The efficiency of the prior art processes is somewhat limited by the presence of claylike components and the selectivity falls off in the smallest particle range of less than 0.1 mm.

**2****DESCRIPTION OF THE INVENTION**

It is therefore an object of the present invention to improve efficiency and selectivity in the process of electrostatically separating particulate mineral mixtures.

Another object of the present invention is an improvement in the efficiency and selectivity of the electrostatic separation of crude potassium salts having a particulate size less than 0.1 mm.

Still another object of the present invention is an improvement in the efficiency and selectivity of the electrostatic separation of crude potassium salts containing impurities of clay.

Other objects of the present invention are improved coatings for particulate mixtures of crude potassium salts which facilitate the electrostatic separation thereof.

A particular object of the present invention is a particulate mixture of crude potassium salt having a coating comprising a mixture of an organic conditioning agent and an inorganic acid or base.

Another particular object of the present invention is a particulate mixture of crude potassium salt that is treated with an inorganic acid or base followed by a treatment with an anionic organic conditioning agent.

Still another particular object of the present invention is a particulate mixture of crude potassium salt that is treated with an anionic organic conditioning agent followed by a treatment with an inorganic acid or base.

A further particular object of the present invention is a particulate mixture of crude potassium salt that is treated with an anionic organic conditioning agent followed by treatment with gaseous hydrogen chloride or ammonia.

Upon further study of the specification and claims other objects and advantages of the present invention will become apparent.

According to the present invention it has been found that the specific distribution of electric charges between the minerals to be electrostatically separated is greatly improved when the powdered mixture, either before, during or after treatment with a prior art conditioning agent, is also treated with very small amounts of inorganic mineral acids, or in other cases with inorganic alkaline reacting substances, preferably NaOH, KOH, or NH<sub>4</sub>OH. Even with mineral mixtures that are difficult to process, it is possible with the present invention to give them strong and highly selective charges. The unfavorable effect of claylike components, which limited the prior art processes, is to a large extent avoided thereby while at the same time the selectivity in the smallest particle range of less than 0.1 mm. diameter is considerably increased.

The acids or bases which are used as additional reagents are applied advantageously as dilute or concentrated solutions in water, but are also added to the mineral mixture in their gaseous or solid state and thoroughly mixed therewith. The most suitable reagent, its most suitable concentration and the best method of adding it, depend largely on the properties of the mineral mixture to be processed and are easily determined by those skilled in the art.

The electrostatic separation of the present invention is advantageously carried out with ground or pulverized particulate mineral crudes such as sylvinite and hartsalz or mixtures thereof with the separation of salts such as sylvite, kierserite, rock salt and halite.

Representative examples of the organic conditioning agents suitable for conditioning the sylvite containing crude salts or mixtures of those crude salts prior to the separation steps are among others:

- (1) Mixtures of fatty acids C<sub>3</sub>–C<sub>22</sub> or of parts thereof, for instance
- Mixtures of fatty acids C<sub>3</sub>–C<sub>10</sub>
  - Mixtures of fatty acids C<sub>6</sub>–C<sub>12</sub>
  - Mixtures of fatty acids C<sub>10</sub>–C<sub>14</sub>
  - Mixtures of fatty acids C<sub>12</sub>–C<sub>18</sub>
  - Mixtures of fatty acids C<sub>14</sub>–C<sub>22</sub>
- (2) Linseed oil fatty acids;
- (3) Benzoic acid;
- (4) Phenylacetic acid;
- (5) Salicylic acid;
- (6) Phthalic acid;
- (7) Alpha-nitroso-beta-naphthol, and salts of the above organic acids;
- (8) Nonyl sulfate;
- (9) Sodium salt of alkylsulfonic acid;
- (10) Sodium salt of oxystearic sulfonic acid;

be construed as merely illustrative, and not limitative of the remainder of the specification and claims in any way whatsoever.

Example 1

- 5 Crude material: Hartsalz with a K<sub>2</sub>O content of 12.9%. Conditioning agent: a first run fatty acid mixture having 6–12 C-atoms.
- The hartsalz is ground to a fineness of less than 1.0 mm. and is first conditioned and mixed by spraying upon it
- 10 0.2 g./kg. of a mixture of, e.g. first run fatty acids having about 6–12 C-atoms and is then warmed to 65° C. by a current of warm air and separated into its components by falling through a potential gradient of 4 kv./cm. in a free-fall electrostatic separator. Instead of the first run fatty acids, other prior art conditioning agents are used, as suggested for example by the German and United States patents disclosed in the Background of the Invention.

TABLE I

| Conditioning Agent                              | Percent K <sub>2</sub> O in residue | Percent K <sub>2</sub> O in 1st concentrate | Percent K <sub>2</sub> O in 2nd concentrate |
|-------------------------------------------------|-------------------------------------|---------------------------------------------|---------------------------------------------|
| 0.2 g./kg. of first run fatty acid mixture..... | 2.5                                 | 25.2                                        | 41.0                                        |

- (11) Sodium salt of benzylnaphthalenesulfonic acid;
- (12) Sulfonated amides of fatty acids;
- (13) Sodium salt of oxystearinsulfonic acid+sodium salt of alkylsulfonic acid 1:1;
- (14) Sodium salt of oxystearic sulfonic acid+sodium salt of ricinic acid 1:1;
- (15) Beta-nitroso-alpha-naphthol and mixtures of 1 to 15.

Preferred examples of the inorganic acids used in the

- 25 Further runs were then performed in which the crude salt after being conditioned with the first run fatty acid mixture was then mixed with 0.5 ml. of two normal acids per kg. of crude salt. After this second mixing the salt was warmed to 65° C. and dried by a current of warm air
- 30 and then separated into its components in the same manner as disclosed above, in a free-fall separator by a potential gradient of 4 kv./cm. The results are given in Table II.

TABLE II

| Conditioning Agent                                                             | Percent K <sub>2</sub> O in residue | Percent K <sub>2</sub> O in 1st concentrate | Percent K <sub>2</sub> O in 2nd concentrate |
|--------------------------------------------------------------------------------|-------------------------------------|---------------------------------------------|---------------------------------------------|
| 0.2 g./kg. first run fatty acid—<br>Plus 0.5 ml./kg. 2 N HCl.....              | 1.1                                 | 40.6                                        | 54.0                                        |
| Plus 0.5 ml./kg. 2 N H <sub>2</sub> SO <sub>4</sub> .....                      | 1.1                                 | 39.3                                        | 51.1                                        |
| Plus 0.5 ml./kg. HNO <sub>3</sub> .....                                        | 1.3                                 | 34.2                                        | 48.9                                        |
| Plus 0.5 ml./kg. H <sub>3</sub> PO <sub>4</sub> .....                          | 0.9                                 | 38.2                                        | 50.8                                        |
| Plus 0.5 ml./kg. 2 N colloidal silicic acid suspended in H <sub>2</sub> O..... | 1.6                                 | 36.0                                        | 51.0                                        |

present invention are HCl in aqueous or gaseous form, H<sub>2</sub>SO<sub>4</sub>, HNO<sub>3</sub>, H<sub>3</sub>PO<sub>4</sub> and colloidal silicic acid suspended in water.

The inorganic bases preferably used in the present invention are aqueous or gaseous NH<sub>3</sub>, NaOH or KOH.

Combinations of mineral mixtures with a conditioning agent and an inorganic acid which particularly illustrate the new and unexpected results of the invention are hartsalz having in terms of K<sub>2</sub>O, 12.9% treated with 6 to 12 carbon atom fatty acid and HCl, H<sub>2</sub>SO<sub>4</sub>, HNO<sub>3</sub>, H<sub>3</sub>PO<sub>4</sub> or colloidal silicic acid; and hartsalz having about 12–13% K<sub>2</sub>O and 3% clay treated with 3 to 12 carbon atom fatty acid mixture, salicylic acid, phenylacetic acid, phthalic acid, or nitroso-beta-naphthol and HCl, H<sub>2</sub>SO<sub>4</sub>, HNO<sub>3</sub> or H<sub>3</sub>PO<sub>4</sub>.

Illustrations of combinations of mineral mixtures with a conditioning agent and an inorganic base showing the new and unexpected results of the present invention include sylvite having in terms of K<sub>2</sub>O, 18.5% and 5% clay treated with 6 to 12 carbon fatty acid and NaOH, KOH, NH<sub>4</sub>OH or NH<sub>3</sub>; and sylvite having 15–16% K<sub>2</sub>O and about 2% clay with 3 to 12 carbon fatty acid, salicylic acid, benzoic acid or phthalic acid and NaOH, KOH or NH<sub>4</sub>OH.

The procedures and conditions for crushing the mineral mixture, applying the conditioning agent and carrying out the electrostatic separation are fully disclosed in U.S. Patents 3,217,876 and 3,225,924.

Before separation in the electrostatic field the preconditioned salts are preferably heated to temperatures between about 30 and 90° C.

Without further elaboration, it is believed that one skilled in the art can, using the preceding description, utilize the present invention to its fullest extent. The following preferred specific embodiments are, therefore, to

- 45 whereas without the subsequent treatment shows the extraordinary improvement in the separating process. Whereas without the subsequent treatment with acid solutions the residues contained about 2.5% K<sub>2</sub>O, the residues after acid treatment contained only 0.9 to 1.6% K<sub>2</sub>O. The improvement is shown even more clearly by the concentrates. After the subsequent acid treatments the K<sub>2</sub>O concentrations were 10–15% higher in the first separation stage than without such acid treatment, and in the second separation stage they were also 10–15% higher. After such acid treatment the highest concentrates (by which is meant the end products of concentration after two or more concentrating stages) show an exceptionally high degree of purity.
- 55 Whereas without acid treatment it is possible in the present case to obtain a maximum concentration of only 52% K<sub>2</sub>O yield of 88%, after the acid treatment a maximum concentration of more than 60% K<sub>2</sub>O with a total K<sub>2</sub>O yield of 92% or more was obtained.

As Table III shows, the selectivity in the fine granular range that is difficult to process is greatly improved by the acid treatment.

TABLE III

65 Selectivity of electrostatic separation in granule size ranges up to 0.1 mm.

| Conditioning                                                   | Granule size ranges                   |
|----------------------------------------------------------------|---------------------------------------|
| 0.2 g./kg. first run fatty acid.....                           | 0–0.06 mm. 28.2                       |
| 0.2 g./kg. first run fatty acid plus 0.5 mg./kg. 2 N acid..... | 0.06–0.1 mm. 44.3 (1) 47.6 57.3 ..... |

1 Percent K<sub>2</sub>O in the highest concentrate.

The results listed in Table IV show that the crude salts that were separated as illustrated in Tables II and III may

have the process modified by subjecting the salts to the acid treatment before as well as after their conditioning treatment with the usual conditioning agents, and also in admixture with the conditioning agents.

TABLE IV

Treatment with the acid before, with or after the addition of the first run fatty acids or the like.

Conditioning agent: First run fatty acid mixture having 6-12 C-atoms.

The crude salt is ground to 1.0 mm. granule size and is first sprayed in with 0.2 g. of a mixture of first run fatty acids having 6-12 C-atoms per kg. of crude salt, and then without subsequent conditioning is warmed to 60° C. by a current of warm air and is then separated by a potential gradient of 4 kv./cm. in a free-fall separator. The separated products are listed in Table VI.

TABLE VI

| Conditioning agent                             | Percent K <sub>2</sub> O in residue | Percent K <sub>2</sub> O in 1st concentrate | Percent K <sub>2</sub> O in 2nd concentrate |
|------------------------------------------------|-------------------------------------|---------------------------------------------|---------------------------------------------|
| 0.2 g. first run fatty acid per kg. crude salt | 4.7                                 | 25.1                                        | 30.5                                        |
| Percent K <sub>2</sub> O in residue            |                                     |                                             |                                             |
| Percent K <sub>2</sub> O in 1st concentrate    |                                     |                                             |                                             |
| Conditioning with mineral acid:                |                                     |                                             |                                             |
| Before                                         | 1.2                                 | 35.1                                        |                                             |
| With                                           | 1.3                                 | 36.2                                        | 20                                          |
| After                                          | 1.1                                 | 39.4                                        |                                             |

The high K<sub>2</sub>O content in the residue and also the meagre enrichment of it in the concentrates show that this is not a good processing method.

TABLE VII

| Conditioning Agent                                                                  | Percent K <sub>2</sub> O in residue | Percent K <sub>2</sub> O in 1st concentrate | Percent K <sub>2</sub> O in 2nd concentrate |
|-------------------------------------------------------------------------------------|-------------------------------------|---------------------------------------------|---------------------------------------------|
| 0.2 g. first run fatty acid mixture per kg. crude salt—                             |                                     |                                             |                                             |
| Plus 0.5 ml. 2 N NaOH per kg. crude salt                                            | 1.9                                 | 38                                          | 49                                          |
| Plus 0.5 ml. 2 N KOH per kg. crude salt                                             | 1.9                                 | 38.8                                        | 50.1                                        |
| Plus 0.5 ml. 2 N NH <sub>4</sub> OH per kg. crude salt                              | 1.6                                 | 40.5                                        | 52.3                                        |
| Plus 0.017 grams gaseous NH <sub>3</sub> per kg. crude salt added to the drying air | 1.5                                 | 42.0                                        | 54.0                                        |

The values given in Table V show that the results depend primarily on the amount of pure acid with which the crude salt is treated, and that the concentration of the acid is of only little importance.

In the separation runs listed in Table V the acid concentrations ranged from 4 N to gaseous, water-free HCl. It is of importance only that the absolute amount of acid is kept at an optimum value, such as can easily be determined by one skilled in the art.

35

In Table VII are given the results of subsequent treatment with diluted alkalies, aqueous ammonia or gaseous ammonia added to the drying air, of the crude salt that has been preconditioned with the fatty acids. In each case there was a definite improvement in the processing. The K<sub>2</sub>O contents of the residues are now only about  $\frac{1}{3}$  as high as without the use of alkalies as ancillary conditioning agents. The K<sub>2</sub>O contents of the concentrates are about 15-25% higher.

TABLE V

| Conditioning Agent               | Percent K <sub>2</sub> O in residue | Percent K <sub>2</sub> O in 1st concentrate | Percent K <sub>2</sub> O in 2nd concentrate |
|----------------------------------|-------------------------------------|---------------------------------------------|---------------------------------------------|
| 0.2 g./kg. first run fatty acid— |                                     |                                             |                                             |
| Plus 0.25 ml. 4 N HCl            | 1.0                                 | 41.0                                        | 55.1                                        |
| Plus 0.125 ml. 8 N HCl           | 1.2                                 | 42.3                                        | 55.0                                        |
| Plus 0.99 ml. 12 N HCl           | 1.1                                 | 41.5                                        | 54.3                                        |

## Example 2

As previously set forth in the specification, applicants have found that in some cases the treatment with inorganic bases is preferred to the treatment with inorganic acid.

50

Crude material: Hartsalz with a K<sub>2</sub>O content of 12-13% and 3% clay.

Separation temperature: 70° C.

## Examples 3a to 3e

Crude material: Hartsalz with a K<sub>2</sub>O content of 12-13% and 3% clay.

Separation temperature: 70° C.

TABLE VIII

| Organic Conditioning agent                                                  | Inorganic acid                                 | Percent K <sub>2</sub> O in 2nd concentrate | K <sub>2</sub> O yield (content of raw material equals 100%) |
|-----------------------------------------------------------------------------|------------------------------------------------|---------------------------------------------|--------------------------------------------------------------|
| (a) Fatty acid mixture of C <sub>5</sub> -C <sub>12</sub> atoms, 0.2 g./kg. | 2 ml./kg. 1 N HCl                              | 41.0                                        | 88                                                           |
| Do                                                                          | 2 ml./kg. 2 N HCl                              | 56.8                                        | 94.8                                                         |
| Do                                                                          | 0.5 ml./kg. 2 N HCl                            | 56.1                                        | 95.4                                                         |
| Do                                                                          | 0.5 ml./kg. 2 N H <sub>2</sub> SO <sub>4</sub> | 54.0                                        | 95.1                                                         |
| Do                                                                          | 0.5 ml./kg. 2 N H <sub>3</sub> PO <sub>4</sub> | 51.1                                        | 94.9                                                         |
| (b) Salicylic acid, 0.2 g./kg.                                              | 0.5 ml./kg. 2 N H <sub>3</sub> PO <sub>4</sub> | 50.8                                        | 94.6                                                         |
| Do                                                                          | 2 ml./kg. 1 N HCl                              | 45.3                                        | 88.2                                                         |
| Do                                                                          | 1 ml./kg. 1 N H <sub>2</sub> SO <sub>4</sub>   | 53.5                                        | 96.5                                                         |
| (c) Phenylacetic acid, 0.2 g./kg.                                           | 2 ml./kg. 1 N HCl                              | 54.1                                        | 93.4                                                         |
| Do                                                                          | 1 ml./kg. 1 N H <sub>2</sub> SO <sub>4</sub>   | 46.5                                        | 85.5                                                         |
| Do                                                                          | 2 ml./kg. 1 N H <sub>3</sub> PO <sub>4</sub>   | 55.3                                        | 93.3                                                         |
| (d) Phthalic acid, 0.2 g./kg.                                               | 2 ml./kg. 1 N H <sub>3</sub> PO <sub>4</sub>   | 45.7                                        | 95.2                                                         |
| Do                                                                          | 2 ml./kg. 1 N HCl                              | 45.1                                        | 85.2                                                         |
| Do                                                                          | 2 ml./kg. 1 N HNO <sub>3</sub>                 | 57.8                                        | 94.5                                                         |
| (e) Nitroso- $\beta$ -naphthol, 0.2 g./kg.                                  | 1 ml./kg. 2 N HCl                              | 55.8                                        | 94.1                                                         |
| Do                                                                          | 1 ml./kg. 2 N H <sub>2</sub> SO <sub>4</sub>   | 46.0                                        | 83.1                                                         |
| Do                                                                          | 1 ml./kg. 2 N H <sub>3</sub> PO <sub>4</sub>   | 53.4                                        | 95.1                                                         |
| Do                                                                          | 1 ml./kg. 2 N HCl                              | 52.9                                        | 94.8                                                         |

It is here shown that treatment with alkalies as ancillary conditioning agents results in a desired improvement. As an example of this, the electrostatic processing of a clay-rich sylvite:

Raw material: Sylvite with a K<sub>2</sub>O content of 18.5% having about 5% clay.

## Examples 4a-4d

Crude material: Sylvite with a K<sub>2</sub>O content of 15-16% and about 2% clay.

Separation temperature: 45° C.

75

TABLE IX

| Organic Conditioning agent                                             | Inorganic Base                     | Percent K <sub>2</sub> O in 2nd concentrate | Exploited K <sub>2</sub> O of the crude salt containing K <sub>2</sub> O |
|------------------------------------------------------------------------|------------------------------------|---------------------------------------------|--------------------------------------------------------------------------|
| (a) Fatty acid mixture of C <sub>5</sub> -C <sub>12</sub> , 0.2 g./kg. | 2 ml./kg. 1 N NH <sub>4</sub> OH   | 30.5                                        | 79.7                                                                     |
| Do.                                                                    | 2 ml./kg. 1 N NH <sub>4</sub> OH   | 56.8                                        | 95.7                                                                     |
| Do.                                                                    | 0.5 ml./kg. KOH                    | 57.1                                        | 96.0                                                                     |
| Do.                                                                    | 0.5 ml./kg. NaOH                   | 50.1                                        | 94.1                                                                     |
| Do.                                                                    | 0.5 ml./kg. NaOH                   | 52.0                                        | 94.7                                                                     |
| (b) Salicylic acid, 0.2 g./kg.                                         | 2 ml./kg. 1 N NH <sub>4</sub> OH   | 46.7                                        | 85.3                                                                     |
| Do.                                                                    | 0.5 ml./kg. 1 N NH <sub>4</sub> OH | 56.3                                        | 94.7                                                                     |
| Do.                                                                    | 2 ml./kg. 1 N NH <sub>4</sub> OH   | 55.8                                        | 94.0                                                                     |
| (c) Benzoic acid, 0.2 g./kg.                                           | 2 ml./kg. 1 N NH <sub>4</sub> OH   | 46.3                                        | 86.3                                                                     |
| Do.                                                                    | 2 ml./kg. 1 N NaOH                 | 55.3                                        | 95.0                                                                     |
| Do.                                                                    | 2 ml./kg. 1 N NaOH                 | 55.1                                        | 94.8                                                                     |
| (d) Phthalic acid, 0.2 g./kg.                                          | 2 ml./kg. 1 N NH <sub>4</sub> OH   | 47.1                                        | 85.8                                                                     |
| Do.                                                                    | 0.5 ml./kg. 1 N NaOH               | 58.8                                        | 93.2                                                                     |
| Do.                                                                    | 0.5 ml./kg. 1 N NaOH               | 56.8                                        | 94.1                                                                     |

The preceding examples can be repeated with similar success by substituting the generically and specifically described reactants and operating conditions of this invention for those used in the preceding examples.

We claim:

1. In a process for electrostatic separation of sylvite containing crude salt mineral, the improvement comprising: contacting said mineral, after grinding, with a small amount of an agent selected from the group consisting of a small amount of aqueous HCl, aqueous H<sub>2</sub>SO<sub>4</sub>, aqueous H<sub>3</sub>PO<sub>4</sub>, aqueous NaOH, aqueous KOH, aqueous NH<sub>4</sub>OH, a suspension of silicic acid in water, gaseous NH<sub>3</sub> or gaseous HCl and additionally conditioning said mineral with organic conditioning agents containing an anionic organic radical and warming up said mineral in a stream of hot drying gas and subjecting said mineral to electrostatic separation of its components.

2. The electrostatic separation process of claim 1, wherein said agent is selected from the group consisting of aqueous suspensions and solutions of inorganic hydroxides.

3. The electrostatic separation process of claim 1, wherein said inorganic acids and bases are selected from the group consisting of about 200-2000 ml. of about 1.0 to 4 normal HCl, about 200-2000 ml. of about 1.0 to 4 normal H<sub>2</sub>SO<sub>4</sub>, about 200-2000 ml. of about 1.0 to 4 normal HNO<sub>3</sub>, about 200-2000 ml. of about 1.0 to 4 normal colloidal silicic acid suspended in water, about 200-2000 ml. of about 1.0 to 4 normal NaOH, about 200-2000 ml. of about 1.0 to 4 normal KOH, about 200-2000 ml. of about 1.0 to 4 normal NH<sub>4</sub>OH, about 5-25 g. gaseous NH<sub>3</sub> or about 5-25 g. HCl per ton salt mineral.

4. The process according to claim 3, wherein said inorganic agents and said anionic conditioning agents simultaneously or after mixing with said ground salt min-

eral are warmed up with hot gas at temperatures between about 30-90° C.

5. The electrostatic separation process of claim 3, wherein said inorganic acids and bases are selected from the group consisting of about 500-2000 ml. of about 1-2 normal HCl, about 500-2000 ml. of about 1-2 normal H<sub>2</sub>SO<sub>4</sub>, about 500 ml. of about 2 normal colloidal silicic acid suspended in water, about 500-2000 ml. of about 1-2 normal NaOH, about 500-2000 ml. of about 1-2 normal KOH, about 500-2000 ml. of about 1-2 normal NH<sub>4</sub>OH, about 5-25 g. gaseous NH<sub>3</sub> per ton salt mineral, or about 5-25 g. gaseous HCl per ton salt mineral, and said salt mineral is conditioned with a small quantity of about 200 g. of an organic anionic conditioning agent per ton salt mineral.

#### References Cited

#### UNITED STATES PATENTS

|    |           |         |          |           |
|----|-----------|---------|----------|-----------|
| 35 | 2,090,418 | 8/1937  | Johnson  | 209-127   |
|    | 2,188,932 | 2/1940  | Weinig   | 209-167 X |
|    | 2,593,431 | 4/1952  | Fraas    | 209-9     |
|    | 3,008,573 | 11/1961 | Gross    | 209-9     |
| 40 | 3,049,233 | 8/1962  | Marullo  | 209-166   |
|    | 3,388,794 | 6/1968  | Peuschel | 209-9     |

#### FOREIGN PATENTS

|           |         |          |
|-----------|---------|----------|
| 650,049   | 10/1962 | Canada.  |
| 1,108,632 | 6/1961  | Germany. |

HARRY B. THORNTON, Primary Examiner

R. HALPER, Assistant Examiner

U.S. Cl. X.R.

50 209-127